

## UNITED STATES PATENT OFFICE

HEINRICH BORSARI-FISCHER, OF ZOLLIKON, NEAR ZURICH, SWITZERLAND  
PROCESS FOR COVERING SURFACES WITH PLATES FROM FUSIBLE MATERIAL AND  
PRODUCT RESULTING THEREFROM

No Drawing. Application filed September 30, 1927, Serial No. 223,248, and in Germany August 8, 1927.

Protective coatings made from mixtures of asphalt, ozocerite, pitches and pitch-like material to which filling substances, such as talc, may be added, were hitherto applied to the surface to be protected, for instance to concrete plates, by adhesive means.

According to the present invention the process for covering the inner walls of vessels with plates of fusible material, such as asphalt mixtures and ozocerite mixtures, is carried out in that a plate cut in accordance with the size of the surface to be coated is "molten on" to the surface under the action of a heating flame effecting a progressive heating. The plate in question may be formed from a warm soft mass by casting or rolling and is cut out according to the predetermined size adapted to the corresponding surface to be coated. When the plates are of great size, they are rolled up into rolls after being suitably sprinkled with talc so as to avoid adhesion and are then cooled down. In this cooled condition the plates may be kept for any desired time or shipped either rolled up or in a flat state. According to the process of the present invention the said plates may also be made up of a normal size and are kept in stock as flat plates. Such plates are flexible to a slight extent even at an ordinary temperature and are applied to the surface to be protected by slight warming, it being obvious that instead of heating the plate also the surface to be coated may be progressively heated, and in a corresponding degree the plate itself is gradually pressed thereon. The procedure of applying the plate in a melting condition to the surface of a wall may suitably be assisted by pressing a wooden or metallic roller thereon. The plate to be applied to has due to the warming a more or less fluid layer which with the assistance of the pressure of the compressional roller is pressed, for instance, against a plastered wall and is thus adapted to be securely kept there-

melting an intimate connection between the individual plates takes place thus ensuring a continuous unitary plane.

What I claim is:

1. The method of covering surfaces with relatively thick layers of a fusible material in a substantially solid condition which comprises applying a layer of said material to the surface to be covered, heating the face of the material in contact with the surface to be covered in order to partially fuse said face, and thereafter pressing the layer against the surface. 55

2. As a new article of manufacture, a surface covered with a relatively thick layer of a fusible material, the face thereof in contact with the surface being fused and pressed against said surface. 65

In testimony whereof I affix my signature.

HEINRICH BORSARI-FISCHER. 70

75

80

85

90

95

100

45 on. Due to the warming required between the surface of the wall and the surface of the plate facing the wall also the edges of the plate already applied to are somewhat heated 50 and when the inner surfaces of the plates are